

July 9, 1929.

E. C. SMITH

1,720,383

INGOT AND MOLD FOR MAKING SAME

Filed Dec. 29, 1924



Fig. 2

INVENTOR.  
Carl C. Smith,

James Stevens Parmee,  
his Atty.

Patented July 9, 1929.

1,720,383

# UNITED STATES PATENT OFFICE.

EARL C. SMITH, OF MASSILLON, OHIO, ASSIGNOR TO CENTRAL ALLOY STEEL CORPORATION, OF MASSILLON, OHIO, A CORPORATION OF NEW YORK.

## INGOT AND MOLD FOR MAKING SAME.

Application filed December 29, 1924. Serial No. 758,511.

The present improvements, relating, as indicated, to the manufacture of ingots, have more particular regard to the casting of steel ingots in molds of special form whereby an 5 ingot possessing various desirable characteristics is produced. One object thus sought to be obtained is an ingot that will cool relatively quickly, driving the "pipe" to the top, with absence of objectionable surface cracking. 10 Particularly in casting ingots of alloy steel it is undesirable to maintain the metal on top molten too long in order to eliminate the piping, for otherwise the alloying ingredients will tend to segregate and the resulting product will not be of uniform character in respect 15 to such ingredients throughout.

To the accomplishment of the foregoing and related ends, said invention, then consists of the mold and product resulting from its 20 use hereinafter fully described and particularly pointed out in the claims; the annexed drawing and the following description set forth in detail certain mechanism embodying the invention, such disclosed means constituting, however, but one of various 25 mechanical forms in which the principle of the invention may be used.

In said annexed drawing:—

Fig. 1 is a top plan view of a mold constructed in accordance with my present improvements; and Figs. 2 and 3 are central vertical sections thereof taken at right angles to each other, the planes of the sections being indicated by lines 2—2 and 3—3, respectively, 35 Fig. 1.

The ingot mold 1 illustrated in the aforesaid figures, in so far as external features are concerned, resembles the one currently in use, and the same is true of the general construction of such mold, which accordingly need not be described in detail. It will be noted that the mold is provided with a pair of opposed ears or lugs 2 whereby it may be engaged by suitable hoisting casting mechanism when it is desired to move the same about or to strip the same from an ingot cast therein; also that the interior opening 3 in the mold decreases in cross-section gradually from the lower to the upper end of said mold. 45 If desired, however, such opening may thus decrease in cross-section in the opposite direction, as in certain well-known types of ingot molds, the feature of present interest in the design or construction of the mold not 50 being limited to either of such two designs.

As best shown in Fig. 1, the opening in question is of general oblong form in cross-section, i. e., it is wider in the plane indicated by the line 2—2 than in a plane at right angles thereto, as indicated by the line 3—3. The 60 cross-section, however, is not strictly rectangular, due to the fact that all four of the inner walls defining the opening are symmetrically fluted, the flutings 4 being of shallow convex form in cross-section and extending from the bottom to the top of the mold, with the re-entrant angles, formed where their edges meet, filleted so as to avoid any sharp angularities in the resultant product. Furthermore, the flutings 4, as shown 65 in Figs. 2 and 3, decrease gradually in width from the one end to the other of the mold, i. e., from the bottom to the top in the case of the particular design of mold selected for the purpose of illustration.

The form of the ingot cast in my improved mold will obviously be the same as that of the open space therein just described, it being noted that the flutings in such ingot will be concave and joined at their edges by rounded 70 projecting corners instead of the convex flutings joined by filleted re-entrant angles at their edges, as in the case of the interior walls of the mold which defines such space. Said ingot, moreover, will be of general 75 oblong shape in cross-section, that is, its section will be thinner on the plane indicated by the line 3—3 than on the plane indicated by the line 2—2, Fig. 1. I thus retain the rapid cooling condition which has been found 80 desirable in the case of the ordinary rectangular ingot, while, due to the fact that the lateral walls of my improved ingot are fluted in the fashion just described, the surface defects that tend to occur in the ordinary rectangular ingot, due to unequal cooling and resultant cracking of such surface, are substantially entirely eliminated. At the same time such oblong fluted ingot retains 85 the handling and rolling advantages of the ordinary rectangular ingot.

Other forms may be employed embodying the features of my invention instead of the one here explained, change being made in the form or construction, provided the elements 90 stated by any of the following claims or the equivalent of such stated elements be employed.

I therefore particularly point out and distinctly claim as my invention:—

1. An ingot mold, characterized by having the opening therein of general oblong form in cross-section, with all of the walls defining such opening longitudinally fluted in a similar manner, with the flutes forming the main portion of the sides of the opening of greater width than the other flutes, substantially as described. 40
2. An ingot mold, characterized by having the opening therein of general oblong form in cross-section, with all of the walls defining such opening symmetrically fluted, the flutings all being of shallow convex form and extending from the bottom to the top of the mold, and the re-entrant angles where the edges of such flutings meet being filleted. 45
3. As an article of manufacture, an ingot of general oblong form in cross-section, all of the lateral walls of said ingot being longitudinally fluted in a similar manner, with the flutes forming the main portion of the sides of the opening of greater width than the other flutes, substantially as described. 50
4. A mold having a chamber provided with four primary side walls at least two of which have a convex contour and four widened corners each provided with three curved salients intervening between the widened corners and the adjacent primary side walls of the mold, substantially as described. 55
5. A primary mold having a chamber provided with four primary convex side walls and four widened corners each provided with three curved salients intervening between the widened corners and the adjacent primary side walls of the mold, substantially as described. 60
6. A mold the lower portion of which absorbs heat from the ingot more rapidly than the upper portion and having a chamber provided with four primary side walls at least two of which have a convex contour and four widened corners each provided with three curved salients intervening between the widened corners and the adjacent primary side walls of the mold, substantially as described. 65
7. A mold having a chamber provided with four primary convex side walls and four broadened corners, each corner comprising a plurality of flutings of shallow convex form, substantially as described. 70
8. A mold having a chamber provided with four primary convex side walls and four broadened corners, each corner comprising a plurality of flutings of shallow convex form, said flutings being connected with curved salients, substantially as described. 75
9. A mold having a chamber provided with four primary side walls at least two of which have a convex contour and four widened corners, each of said widened corners comprising adjacent convex shallow flutings connected by curved salients, substantially as described. 80
10. A mold having a chamber provided with four primary convex side walls and four broadened corners, each corner comprising a pair of flutings of convex contour projecting inwardly toward the center of the mold cavity in a manner similar to the four primary side walls, said flutings being connected with curved salients substantially as described. 85

Signed by me, this 22nd day of April, 1922.  
EARL C. SMITH.